

May 23, 1950

J. F. SETTLE  
ELECTRICAL CONTACT MEMBER AND  
METHOD OF MAKING THE SAME  
Filed Sept. 12, 1946

2,509,021



Inventor:  
Joseph F. Settle,  
by Powell S. Mack  
His Attorney.

## UNITED STATES PATENT OFFICE

2,509,021

ELECTRICAL CONTACT MEMBER AND  
METHOD OF MAKING THE SAMEJoseph F. Settle, Schenectady, N. Y., assignor to  
General Electric Company, a corporation of  
New York

Application September 12, 1946, Serial No. 696,551

1 Claim. (Cl. 171—326)

**1**  
My invention relates to electrical contact members and to an improved method of making the same.

An object of my invention is to provide an improved electrical member.

Another object of my invention is to provide an improved method of making an electrical contact member.

A further object of my invention is to provide an improved electrical contact brush member having a carbonaceous material portion and an arrangement for securing a terminal clip member thereto.

Further objects and advantages of my invention will become apparent and my invention will be better understood from the following description referring to the accompanying drawing, and the features of novelty which characterize my invention will be pointed out with particularity in the claim annexed to and forming a part of this specification.

In the drawing, Fig. 1 is a sectional side elevational view of a part of an electrical contact member formed as a brush for electrical rotating machinery provided with an embodiment of my invention; and Fig. 2 is a sectional side elevational view of a part of the arrangement shown in Fig. 1 prior to the final assembly thereof.

Referring to the drawing, I have shown my invention in connection with an electrical contact member formed as a brush adapted to be used to make a connection between a stationary conductor and a rotating electrical device. This contact brush member is shown as having a portion 1 made of carbonaceous material, such as graphite or a mixture of graphite and metal powders, or of similar materials, as are conventionally used for such members, and an arrangement is provided for forming a good electrical contact between the contact brush member and a stationary terminal through a flexible electrical conductor 2 which is welded, brazed, or otherwise suitably secured to a terminal clip member 3 of any suitable material, such as steel, arranged over an end and in contact with a surface of the carbonaceous material brush portion 1. In order to provide a secure connection between the terminal clip member 3 and the carbonaceous material brush portion 1, a passage 4 is preformed in the carbonaceous material brush portion 1 and a passage 5 is similarly preformed in the contact clip member 3. The terminal clip member is then arranged over an end of the carbonaceous material brush portion with the two passages 4 and 5 substantially in coaxial correspondence, as

**2**  
shown in Fig. 2, and then a two-part rivet is arranged in the passages 4 and 5 with stem portions 6 and 7 of the two parts of the rivet extending through the members 1 and 3 in the openings 5 and 5 with heads 8 and 9 of the rivet part in engagement with the opposite outer side of the carbonaceous material brush portion and the terminal clip member. When these parts are thus assembled, the two parts of the rivet are adapted to be welded together by the passage of an electric current therethrough, such that the inner adjacent ends 10 and 11 of the two rivet parts are welded together by the passage of current therethrough to provide a rigid unitary rivet securing 10 together the terminal member and the carbonaceous material brush portion 1. When the rivet cools, the contraction thereof assists in providing a still firmer connection between the terminal clip member 3 and the brush member portion 1. This 15 mechanical connection may be further strengthened, and the electrical resistance of the contact between the terminal clip member 3 and the carbonaceous material brush member portion 1 may be reduced by providing a bonded coating 13 of 20 low electrical resistance metal, such as copper, on the surface of the carbonaceous material brush member portion 1 adapted to be arranged in contact with the terminal clip member 3 and applying an adherent coating of an alloying metal, 25 such as tin or zinc, over the surface of the clip member 3 prior to assembly. These two alloying metals are adapted to be alloyed together to provide a low resistance bond between the metal of the clip 3 and the carbonaceous material portion 1 of the brush member by the heat generated 30 by the passage of current through the two parts of the rivet during the welding thereof and by the passage of current through the carbonaceous material brush portion 1 and the clip member 35 during this rivet-welding operation. This alloying of the two contact metals is facilitated by the application of a non-corrosive flux, such as a mixture of rosin and alcohol, over the surface of the alloying metal and particularly over the 40 surface of the copper coating in order to remove the oxide from the engaging surfaces of the alloying metals and to facilitate thereby the wetting of these adjacent surfaces when the metals become molten. This provides a good electrical and mechanical bond between the terminal clip member 45 3 and the carbonaceous material brush member portion 1 by the secure unitary riveted construction of the two-part welded rivet and by the continuous good electrical contact between the steel clip 3, the tin surface thereon, the alloy of the 50 55

tin and copper, the copper surface, and the carbonaceous material 1, forming a good steel-to-tin-to-alloy-to-copper-to-carbonaceous material electrical conductor of relatively low resistance reinforced by the rivet which extends therebetween where these or other suitable electrically conductive members are used in making these parts.

While I have illustrated a particular embodiment of my invention, modifications thereof will occur to those skilled in the art. I desire it to be understood, therefore, that my invention is not to be limited to the particular arrangement disclosed, and I intend in the appended claim to cover all modifications which do not depart from the spirit and scope of my invention.

What I claim as new and desire to secure by Letters Patent of the United States is:

An electrical contact brush having a carbonaceous material portion and a metal terminal clip member adapted to be arranged in contact with a surface of said carbonaceous material portion, said carbonaceous material portion having a coating of copper on the surface thereof adapted to be arranged adjacent said clip member and said

18

10

15

25

metal clip member having a coating of tin on the face thereof arranged to be adjacent said carbonaceous material portion, a two-part rivet extending through both said terminal clip member and said carbonaceous material portion with a head on the outer end of each of said rivet parts and with the adjacent inner ends of said two rivet parts welded together to form a unitary rivet for securing together said terminal clip member and said carbonaceous material brush portion with the heat of said weld forming an alloy between said tin and said copper coatings.

JOSEPH F. SETTLE.

#### REFERENCES CITED

The following references are of record in the file of this patent:

#### UNITED STATES PATENTS

|    | Number    | Name              | Date          |
|----|-----------|-------------------|---------------|
| 20 | 661,669   | Rohrer            | Nov. 13, 1900 |
|    | 1,210,029 | Auel              | Dec. 26, 1916 |
|    | 2,242,014 | Martin            | May 13, 1941  |
|    | 2,436,852 | Carmichael et al. | Mar. 2, 1948  |